

R. HALEY.

GLASSWARE AND METHOD OF DECORATING THE SAME

APPLICATION FILED OCT. 21, 1915.

1,178,257.

Patented Apr. 4, 1916.

FIG.1. 2



FIG.2.



FIG.3. 4 2



FIG.4.



FIG.5.

WITNESSES

J. Herbert Bradley

Ella McConnell



INVENTOR

Ruben Haley,  
By J. Herbert Atty.

# UNITED STATES PATENT OFFICE.

REUBEN HALEY, OF BEAVER, PENNSYLVANIA, ASSIGNOR, BY DIRECT AND MESNE ASSIGNMENTS, OF ONE-HALF TO UNITED STATES GLASS COMPANY, OF PITTSBURGH, PENNSYLVANIA, A CORPORATION OF PENNSYLVANIA, AND ONE-HALF TO THE DUNCAN & MILLER GLASS COMPANY, OF WASHINGTON, PENNSYLVANIA, A CORPORATION OF PENNSYLVANIA.

## GLASSWARE AND METHOD OF DECORATING THE SAME.

1,178,257.

Specification of Letters Patent.

Patented Apr. 4, 1916.

Application filed October 21, 1915. Serial No. 57,155.

*To all whom it may concern:*

Be it known that I, REUBEN HALEY, a citizen of the United States, and resident of Beaver, in the county of Beaver and State of Pennsylvania, have invented certain new and useful Improvements in Glassware and Method of Decorating the Same, of which the following is a specification.

The object of this invention is to provide glassware of novel form, also an efficient method of decorating the same wherein the advantages incident to both pressing and cutting are availed of in one and the same decorative configuration.

15 The brilliancy of fire-finished pressed ornamentation, particularly when sunk deeply into the surface, is well known, and by the invention herein, ornamentation of this character is combined or blended with cut surfaces in such manner as to produce a highly decorative and artistic effect.

20 In the accompanying drawings, Figure 1 is an elevation of a portion of an article of glassware in which the pressed portion of the configuration is formed simultaneously with molding such articles, and Fig. 2 is a section taken on line 2—2 of Fig. 1. Fig. 3 is an elevation similar to Fig. 1, showing the same configuration subsequent to the 25 cutting operation, and Fig. 4 is a section on line 4—4 of Fig. 3, illustrating such operation. Fig. 5 is a cross-section on line 5—5 of Fig. 3.

30 Referring to the drawings, the glass article of which A is a fragment is pressed in manner well known in the art and is subsequently fire-polished, a step equally familiar in the manufacture of glassware, the slight remelting of the surfaces incident to fire-polishing smoothing and imparting thereto a brilliant luster.

35 This invention may be variously practised. In the preferred procedure, the mold in which the article or blank is pressed is formed with the design in raised outline, whereby such configuration is imparted to, *i. e.*, pressed into, the surface of the article. In pursuance of the present invention, portions of this configuration, such as B, are 40 relatively shallow and are subsequently cut, or "recut" as expressed in the trade. Other

portions C of the configuration are relatively deep, these being the portions which appear unchanged in the completed embellishment. After the article has been thus pressed, it is 55 fire-polished, thereby imparting the requisite luster to the undecorated surface portions as well as to the deeper and permanent portions C of the pressed configuration.

50 Pressed and fire-finished blanks of the above description comprise articles of manufacture which are sold by the manufacturer to producers of cut glass or "cutting shops," so-called. Or, the manufacturer of the blanks may cut them and market the finished 55 product.

The cutting of the shallower depressed portions B is accomplished in the usual manner by a cutting wheel W. The cut embellishment may take various forms. In that 70 shown in Figs. 3 and 4, the cut surfaces present minute ridges or ribbing, as indicated at B', this being only one of various effects that may be produced. The cutting of a glass surface always leaves such surface 75 opaque or of frosted appearance, and in practising the present invention this appearance may be maintained, or if preferred it may be removed and a clear luster produced by polishing. The effects thus produced in 80 cut glass are well understood in the art and no novelty is claimed therefor, and are simply referred to as illustrating adaptations of which the present invention is capable.

In the finished article, the deeper portions 85 C retain their pressed outline, as well as their brilliancy resulting from the fire finish. The pressed and cut formations thus combine and blend in producing a highly artistic effect. In the design illustrated, the 90 deeper portions have the appearance of crystal-like oval drops within the surrounding cut portion, the latter by preference, though not necessarily, retaining the opaque or frosted effect produced by cutting. 95

90 The shallower depressed portions are of such form in the direction in which the cutting proceeds as to afford the periphery of the cutting wheel access thereto. As here shown, the surface to be cut is curved in 100 the direction of cutting, and the arc of such curvature corresponds to the peripheral

curvature of the wheel, whereby the latter may enter and resurface or recut the same. The radius of the pressed depression may be greater than that of the wheel, but this is 5 not objectionable as in such case the blank is so moved or "rolled" on the wheel during the cutting operation as to expose all portions of the depression thereto.

When the cut and pressed configurations 10 are combined as shown in the present embodiment, wherein the cut or recut portions surround and constitute a field for the deeper pressed portions, such deeper portions are of such form, at least in the direction of 15 cutting, as to prevent the wheel from entering. By this means the configuration may be cut on all sides or all around depressions C, and in fact the wheel may operate over or cover said depressions, as shown in Fig. 20 4, without interfering therewith or impairing their luster.

In the preferred practice, the deeper depressions C are each shorter and of sharper curvature in the direction of cutting than 25 are depressions B. However, the deeper depressions as well as the surface portions to be cut are not necessarily of the form shown, the invention contemplating any surface arrangement whereby cutting by means of a 30 wheel may proceed adjacent to or over the deeper portions without marring the latter.

I claim:

1. A glass blank provided with surface 35 depressions of different depths, the shallower depressions surrounding and constituting a field for the deeper depressions, the deeper depressions being fire-polished and inaccessible to a cutting tool used for cutting the surfaces of the shallower depressions.

2. A glass article formed with depressions 40 of different depths, the deeper depressions having their surfaces fire-finished and the shallower depressions surrounding the 45 deeper depressions and having their surfaces cut and constituting a field for the fire-finished depressions, thereby providing

a decorative scheme embodying both fire-finished and cut surfaces.

3. The method herein described of decorating glassware, consisting in shaping a glass article and simultaneously forming the surface thereof with a depressed configuration—portions of which are deeper than the remainder, the shallower portions being 55 of predetermined shape in the direction in which they are subsequently cut and the deeper portions having less surface area in said direction than the shallower portions, and cutting the shallower portions on a 60 curved cutting surface of such peripheral area as not to enter the deeper depressions.

4. The method herein described of decorating glassware, consisting in shaping a glass article and simultaneously forming the surface thereof with a depressed configuration, 65 portions of such configuration being deeper than the remainder thereof, the deeper and shallower portions each of curved formation in the direction of subsequent cutting with 70 the curvature of the shallower portions flatter than that of the deeper portions, and grinding and thereby imparting ultimate finish to the shallower portions by means of a grinding surface which is flatter than the 75 curvature of said deeper portions whereby the shallower portions are cut without cutting said deeper portions.

5. The method herein described of decorating glassware, consisting in shaping a glass 80 article and simultaneously therewith forming the surface thereof with depressed configuration, portions of the configuration being deeper than and located within the shallower portions thereof and inaccessible to 85 an implement adapted for cutting the shallower portions, and cutting the shallower portions with such implement.

In testimony whereof I affix my signature in presence of two witnesses.

REUBEN HALEY.

Witnesses:

HARVEY WILSON,  
JOSEPH W. BYERS.

Copies of this patent may be obtained for five cents each, by addressing the "Commissioner of Patents, Washington, D. C."